

# UNITED STATES PATENT OFFICE.

ADOLF SWOBODA, OF VIENNA, AUSTRIA-HUNGARY, ASSIGNOR OF ONE-HALF TO THE FIRM OF ENZESFELDER MUNITIONS- UND METALLWERKE ANTON KELLER AKT. CES., OF VIENNA, AUSTRIA-HUNGARY.

## STRIKING-SURFACE ON SAFETY-MATCH BOXES, &c.

949,920.

Specification of Letters Patent. Patented Feb. 22, 1916.

No Drawing.

Application filed January 30, 1909. Serial No. 475,100.

*To all whom it may concern:*

Be it known that I, ADOLF SWOBODA, a subject of the Emperor of Austria-Hungary, and residing at 60 Geblergasse XVII, Vienna, 5 Austria-Hungary, have invented new and useful Improvements in the Production of Striking-Surfaces on Safety-Match Boxes, Candle-Boxes, and the Like, of which the following is a specification.

10 Hitherto the friction or striking surfaces on boxes particularly boxes for safety matches, that is to say, matches that can be only ignited on a special surface, have been formed by applying the friction substance to the paper that was put around the box. The disadvantage of this method was that when the striking surface became damp the paper layer became spongy and wrinkled and could be easily detached from the wooden 15 surface, so that when a match was struck it was torn off. Moreover the friction surface which had become damp did not easily dry, as the moisture penetrated the layer beneath or was absorbed thereby.

20 According to the present invention a coating substance is produced, which resists moisture and notwithstanding moisture is not destroyed when used. This result is effected by the employment of a bed or 25 ground of gypsum, cement or similar bodies capable of binding, to which the usual substance on which the match is struck and which causes the ignition is applied. This bed or ground forms a firm under-layer 30 which cannot be affected by dampness and therefore prevents the igniting coating being torn off when the match is struck. It thus insures economy in the coating substance.

35 The method is carried out in the following manner. 60 parts of glue size are dissolved in 250 parts of lukewarm water; 60 parts of Portland cement, 60 parts of gypsum, 60 parts of pipe clay, 5 parts of cork 40 meal and 10 parts of iron-minium in the form of fine dry powder are then thoroughly mixed. This mixture is introduced into the glue size solution and stirred therein by means of stirring disks, the solution being 45 kept in a lukewarm state, in order that the size may remain fluid. The substance so

obtained is well ground in a wet mill and subsequently applied in the cold state to the bare wooden surface of the box in the known manner and finally dried until the coating 55 material for igniting the matches can be applied to the bed or ground substance. As a covering for this bed or ground material a mixture consisting of 100 parts of water, 18 parts of mucilage consisting of a solution of 33 parts gum in 67 parts water, 26 parts of amorphous phosphorus, 1 part of finely powdered cork, 10 parts of rye meal and 10 parts of iron minium will be found very effective, this mixture being stirred in 60 a cold state, and ground and worked also in a cold state. It is applied to the bed or ground material in the known manner. Any other material employed hitherto for the purpose may however be applied to my new 65 composition constituting the bed or ground substance.

Having thus described my invention, what I claim is:-

1. The herein described composition of 75 matter for constituting a ground substance for the ignition surfaces of safety match boxes, comprising glue size, cement, gypsum, pipe clay, cork meal, and iron minium, substantially as described.

2. The herein described composition of matter constituting a ground substance for the ignition surfaces of safety match boxes, consisting of approximately equal parts glue size, cement, gypsum, and pipe clay, and 80 relatively smaller parts of cork meal and iron minium, mixed with water, substantially as described.

3. The herein described composition of 85 matter for constituting a ground substance for the ignition surfaces of safety match boxes, consisting of, by weight, 60 parts glue size, 60 parts powdered cement, 60 parts gypsum, 60 parts pipe clay, 5 parts cork meal, 10 parts iron minium, and 250 parts 90 water, substantially as described.

In testimony whereof I affix my signature in presence of two witnesses.

ADOLF SWOBODA.

Witnesses:

ROBERT W. HEINGARTNER,  
JANEZ KNARELJ CACHALY.